

## 1

2,956,880

**PREPARATION OF WASHED EMULSIONS AND GELATIN DERIVATIVES EMPLOYED AS PEPTIZERS IN THEIR PREPARATION**

John W. Gates, Jr., and Paul E. Miller, Rochester, N.Y., assignors to Eastman Kodak Company, Rochester, N.Y., a corporation of New Jersey

No Drawing. Filed Jan. 4, 1957, Ser. No. 632,422

2 Claims. (Cl. 96—94)

This invention relates to the preparation of new gelatin derivatives and the use of those derivatives in the coagulation washing of photographic emulsions in the presence of heavy metal salts.

It is often desirable in the preparation of photographic emulsions that a small amount of a heavy metal salt be incorporated therein to impart desired characteristics to the emulsion. For instance, emulsions are sometimes prepared with cadmium salts, such as cadmium chloride, therein which has the effect of restricting the grain growth in the preparation of the silver halide and also acts as an anti-fogant in the photographic emulsion. The presence of other heavy metal salts such as iron, lanthanum, zinc, aluminum, nickel or chromium, may be desirable in emulsion preparations. Methods for the coagulation washing of photographic emulsions have been described in U.S. Patents Nos. 2,614,928 and 2,614,931. In those methods gelatin derivatives are employed which make possible the conversion of the silver halide dispersion to a coagulated form upon adjustment of the pH thereof. However, when heavy metal salts are present in the emulsion, coagulation of the peptizer may occur at normal pH values. A method for the coagulation washing of emulsions is described in U.S. application Serial No. 406,061 of Russell in which those salts are added to cause coagulation to occur. This method, however, precludes the preparation of the silver halide in the presence of the heavy metal salt to form a silver halide dispersion and therefore is not adapted for use in cases where the presence of the heavy metal salt is desirable in the silver halide formation operation.

One object of our invention is to provide a method of coagulation washing of silver halide dispersions in which heavy metal salts have been employed in their preparation. Another object of our invention is to provide gelatin derivatives which are useful in such a process. A still further object of our invention is to provide a procedure for preparing those gelatin derivatives. A still further object of our invention is to provide a coagulation method in which the coagulation occurs at a pH of 3.0—4.5. Other objects of our invention will appear herein.

We have found that a phthalated gelatin which contains 3—10 percent of a lower fatty acid radical therein such as acetyl, propionyl or the like, may be prepared by reacting phthalyl gelatin with lower fatty acid anhydride or by reacting upon gelatin simultaneously with phthalic anhydride and the lower fatty acid anhydride. We have found that silver halide dispersions in which gelatin derivatives of that type are present, are readily coagulated upon lowering of the pH thereof even though soluble heavy metal salts are present in the silver halide dispersion. We have found that by our procedure washed silver halide emulsions having a heavy metal salt content may be prepared by a coagulation method. The amount of phthalyl added to the gelatin may vary but if the gelatin is reacted with five parts of phthalic

## 2

anhydride per 100 parts of gelatin sufficient phthalyl content is imparted thereto to be suitable for coagulation washing as described herein.

When a gelatin derivative, such as a phthalic anhydride derivative of gelatin prepared by reacting upon 100 parts of gelatin with five parts of phthalic anhydride, is employed as the peptizer for silver halide in a dispersion containing cadmium chloride or the like, this dispersion coagulates at a pH between 7.0 and 4.5. If on the other hand a gelatin derivative containing both phthalyl and acetyl is employed and the silver halide is prepared in the presence of cadmium chloride, no coagulation occurs within this pH range and to obtain coagulation it is necessary to reduce the pH such as to 3.0—4.5. This holds true with gelatin derivatives having various phthalyl contents. For instance, if the gelatin has been reacted with phthalic anhydride in the amount of five parts, seven parts or ten parts thereof per 100 parts of gelatin, the products obtained when used as peptizers will result in coagulation of the silver halide dispersion when cadmium chloride is added at a usual pH; whereas if a small percentage of lower fatty acid radical is present therein, such as 5 percent, 8 percent or 10 percent acetyl, the dispersion does not coagulate when heavy metal salt is present therein. In the latter case, it is only when the pH is reduced to a value within the range of 3.0—4.5 that coagulation occurs.

The coagulate may be washed any number of times at the lowered pH and may be redispersed in water having a pH in the vicinity of 7.0 to form a washed emulsion having a content of heavy metal salt therein. Sometimes it is desirable to add heavy metal salts as coating addenda to emulsions just prior to coating. In those cases with the previously mentioned types of gelatin derivatives used as peptizers, there is danger of haze developing in the emulsion unless a considerable quantity of gelatin was employed as the carrier for the silver halide. By using a peptizer in accordance with our invention, any such haze effect is avoided.

40 The following examples illustrate the preparation of gelatin derivatives useful for preparing washed emulsions in accordance with our invention:

*Example 1*

45 100 parts of 5 percent phthalyl gelatin was plumped for 1 hour in 700 parts of water. The mass was stirred at 110° F. whereupon the gelatin derivative melted. The pH was adjusted to 9.5 with 20 percent aqueous sodium hydroxide. Eighteen parts of propionic anhydride was 50 added dropwise to the stirred mass over a 10-minute period while keeping the pH at 9.5. When the addition of propionic anhydride had been completed, the pH was lowered to 6.0 with 6-N-sulfuric acid. The gelatin derivative thus obtained was chilled, washed and 55 dried in the usual manner. A gelatin derivative having both propionyl and phthalyl groups was obtained. When a solution of this gelatin derivative was mixed with a cadmium chloride solution, no interaction took place, but a coagulate formed upon dropping the pH thereof to 3.8.

*Example 2*

The same procedure as described in the preceding example was employed but 400 parts of 7 percent phthalyl gelatin in 1600 parts of water was employed and this solution was reacted with 100 parts of acetic anhydride at a pH of 9.5. The pH was then adjusted to 5.8. The gelatin derivative obtained was chilled, washed and dried in the usual manner. The gelatin derivative obtained which contained both acetyl and phthalyl groups did not interact with cadmium chloride solution at that pH but upon reducing the pH such as to 3.6, a coagulate was obtained.

## Example 3

A gelatin derivative was prepared by the same procedure as described in Example 1 except that 600 parts of 5 percent phthalyl gelatin was employed in 2400 parts of water and this solution was treated with 120 parts of acetic anhydride at a pH of 9.5. The mass was then adjusted to a pH of 6.0 and the gelatin derivative obtained was chilled, washed and dried in the usual manner. The acetyl phthalyl gelatin did not interact with cadmium chloride solution at that pH but coagulated when the pH was reduced to 3.5.

## Example 4

200 parts of gelatin were plumped in 800 parts of water and a solution was obtained by heating to 110° F. with gentle agitation. The pH was adjusted to 9.5 with 20 percent aqueous sodium hydroxide and 20 parts of finely divided phthalic anhydride was added. The pH was held at 9.5 by the occasional addition of alkali. At the completion of the reaction, 25 parts of acetic anhydride was added dropwise to the stirred solution while maintaining the pH at 9.5. The pH was then adjusted to 6.0 with 6-N-sulfuric acid and the solution was chilled, noodled and washed and the product was dried in a conventional manner. A gelatin derivative containing phthalyl and acetyl groups was obtained.

## Example 5

This derivative was prepared by the same procedure as described in Example 4 using 200 parts of gelatin, 6 parts of phthalic anhydride and 40 parts of acetic anhydride. The gelatin derivative obtained contained both acetyl and phthalyl groups. It had useful properties for the preparation of washed emulsions containing heavy metal salts in which the emulsions could be coagulated at a pH within the range of 3.4-4.0.

The following example illustrates the preparation of a washed photographic emulsion having therein a heavy metal salt and employing as the peptizing agent an acetylated phthalylated gelatin.

## Example 6

Into a container with temperature control was put a solution with the following composition:

|                                                                                                                             | Parts |
|-----------------------------------------------------------------------------------------------------------------------------|-------|
| Potassium bromide                                                                                                           | 165   |
| Potassium iodide                                                                                                            | 5     |
| Acetyl phthalyl gelatin prepared using 7 parts of phthalic anhydride per 100 of gelatin and having an acetyl content of 10% | 50.5  |
| Cadmium chloride                                                                                                            | 7.5   |
| Water                                                                                                                       | 1700  |

In another container a filtered solution consisting of 200 parts of silver nitrate and 2000 parts of water was placed. The silver nitrate solution was placed in a separating funnel at a temperature of 72° C. from which it was run, slowly, through a calibrated nozzle into the first container. The contents of the latter were kept at a temperature of 70° C. and in constant motion by a mechanical stirrer during the precipitation and ripening.

An emulsion was prepared in the absence of cadmium chloride using the same amount of phthalyl gelatin derivative, which derivative had no acetyl therein. The pH of the respective emulsions was lowered by the addition of sulfuric acid to the point at which the silver halide dispersions coagulated, the mother liquor was decanted off in each case and the silver halide dispersion was washed twice at 20° C. There was then added to the mass sufficient gelatin in distilled water to form a satisfactory emulsion upon stirring the mass at 40° C. Ammonia was added to bring the emulsion pH to 6.5 and

stirring was continued until all of the solid matter was completely dispersed.

The two emulsions thus prepared were coated in the conventional manner upon suitable film base, exposed  $\frac{1}{25}$  of a second using an Eastman 1B sensitometer with a 500-watt lamp at 3000° K. and developed 4 minutes in Kodak developer D-19. The emulsion in which the cadmium chloride was employed had a similar speed and a higher gamma value than that in which the cadmium chloride was omitted. The addition of cadmium chloride to the dispersion prepared using nonacetylated phthalyl gelatin causes coagulation during the formation of the silver halide and therefore the emulsion cannot be prepared.

In the above description, the phthalyl percentage is given in terms of the percent of phthalic anhydride employed in preparing the derivative based upon the weight of the gelatin. The method described in Yutzy and Frame Patent No. 2,525,753 is a typical example of the preparation of the phthalylated gelatin. By this method sufficient phthalyl is imparted to the gelatin to impart acid-reversible characteristics thereto. The amount of fatty acid radical imparted to the gelatin to give the desired effect in accordance with our invention is 3 percent up to 10 percent or even more if esterifiable groups are present in the gelatin. The amount of cadmium chloride or other heavy metal salt which is present in the emulsion in accordance with our invention may be from  $\frac{1}{4}$  percent up to 4 percent based on the weight of the gelatin employed. The coagulation values for the silver halide dispersions which are coagulated in accordance with our invention are all found within the range of 3-4.5. The acetyl phthalyl gelatins prepared in accordance with our invention are obtained either by acylating phthalyl gelatin or by reacting upon gelatin with both phthalic anhydride and lower fatty acid anhydride simultaneously. The gelatin which is employed is preferably of photographic grade.

We claim:

40. 1. A method of preparing a silver halide dispersion adapted to be coagulation washed even in the presence of heavy metal salts which comprises reacting alkali metal halide with silver nitrate in an aqueous solution containing the soluble salt of a polyvalent heavy metal and as the peptizing agent therein gelatin lower alkanoate phthalate which is the reaction product of a lower alkanoic acid anhydride and phthalic anhydride with gelatin in the ratio of 5 to 20 parts by weight of the lower alkanoic acid anhydride, 3 to 10 parts by weight of the phthalic anhydride and 100 parts by weight of the gelatin.
45. 2. A method of preparing washed silver halide photographic emulsion which comprises mixing in the presence of cadmium chloride a solution of silver nitrate and as a peptizer a solution of alkali metal halide with a gelatin acetate phthalate which is a reaction product of acetic acid anhydride and phthalic anhydride with gelatin in the ratio of 5 to 20 parts by weight of acetic acid anhydride, 3 to 10 parts by weight of phthalic anhydride and 100 parts by weight of gelatin, thereby forming a silver halide dispersion, adding acid to the dispersion to reduce the pH of the mass to a value within the pH range of 3-4.5 to coagulate the solids therein and subsequently dispersing the coagulate in a vehicle for the silver halide under non-coagulating conditions.

## References Cited in the file of this patent

## UNITED STATES PATENTS

- |           |                    |               |
|-----------|--------------------|---------------|
| 2,423,773 | Hart et al. -----  | July 8, 1947  |
| 2,494,041 | Frame -----        | Jan. 10, 1950 |
| 2,592,263 | Frame -----        | Apr. 8, 1952  |
| 2,614,928 | Yutzy et al. ----- | Oct. 21, 1952 |
| 2,614,929 | Yutzy et al. ----- | Oct. 21, 1952 |